

Patented Mar. 30, 1926.

1,578,376

# UNITED STATES PATENT OFFICE.

FRITZ SEIDENSCHNUR, OF FREIBERG, GERMANY.

## METHOD FOR THE PRODUCTION OF COKE AND TAR FROM COAL.

No Drawing.

Application filed October 2, 1924. Serial No. 741,286.

*To all whom it may concern:*

Be it known that I, FRITZ SEIDENSCHNUR, a citizen of Germany, residing at Freiberg, in the State of Saxony, Germany, have invented certain new and useful Improvements in a Method for the Production of Coke and Tar from Coal: and I do hereby declare the following to be a full, clear, and exact description of the invention, such as will enable others skilled in the art to which it appertains to make and use the same.

My invention has for its object a method for the production from mineral coal of a tar, stiff at ordinary temperatures and rich 15 in undecomposed bitumen, simultaneously with the production of a coke which is rich in readily inflammable gases.

In the German patent specification 372,244 a method and means are given for the production of a tar from wet lignite, which is stiff at ordinary temperature and becomes liquid at a temperature of over 30-40° C., said tar being rich in undecomposed bitumen. By carrying out this method a coke 20 rich in gases and readily inflammable may also be obtained from the lignite, which, as proved by actual experiments on renewed heating to about 500° C. gives off a multiple of the amount of combustible gaseous substances which are developed from ordinary 25 commercial coke by such treatment. Such coke, obtained from lignite, which is readily inflammable and rich in gases is quite correctly termed "lignite-flame coke" on account 30 of its suitability to burn with a flame due to its richness in gas, in any appropriate grate.

In an effort to make use of the continuous working method according to German patent 40 specification No. 372,244 for mineral coal, doubts have arisen as to its applicability.

Firstly it seemed questionable whether a tar stiff at ordinary temperatures and rich in undecomposed bitumen could be obtained at 45 all since, for example, with the means hitherto employed for extracting bitumen (more or less complete) from lignite scarcely any success had been obtained with mineral coal. Moreover while the large quantities of steam necessary for the liberation of a tar rich in 50 bitumen are not available when working mineral coal, yet the co-action of said steam with lignite is considered to be essential to cause the separation of the bitumen of the lignite in a nearly undecomposed form. The 55 fundamental differences in the properties

of mineral coal and lignite were per se opposed to the production of a coke rich in gas from mineral coal of a quality similar to the above-mentioned lignite flame-coke 60 with the avoidance as far as possible of combustible gases; to this had to be added the development of relatively large gas-quantities by the usual production of crude tar in a rotary furnace and, finally, also the inclination of a mineral coal rich in tar to fuse and bake together by treatment with hot gases, for example in a slow combustion generator. It is well known that, in spite of repeated stoking or the addition of lignite, 70 a continuous working can hardly be maintained in a generator. Consequently experiments aimed at obtaining by means of slow combustion, products from mineral coal of the same high value as from lignite, did not 75 possess much possibility of success.

It came therefore as a surprise when it was found that a stiff tar and a flame-coke free of tar and rich in readily inflammable gases could in fact be obtained from mineral coal by treatment with hot gases which are free of oxygen and are employed in larger quantities than those which have been found sufficient for the production of a tar and flame-coke from lignite according to 80 German Patent No. 372,244.

Whereas according to Fischer's treatise entitled "Gesammelte Abhandlungen zur Kenntniss der Kohle" volume III, page 212, crude tar produced in the usual manner from 85 mineral coal is liquid at normal temperatures, the setting point of the tar rich in bitumen and produced in the aforesaid manner is at about 30° C.; also its viscosity and the amount of paraffin wax are correspondingly higher if the stiff tar is subjected to a 90 further distillation treatment.

The flame-coke, free of tar, obtained from mineral coal, by heating to about 500° C. in a "Fischer" aluminum and slow-combustion apparatus, develops about 1 litre of a highly valuable gas, very rich in methane (each 20 gr. substance) whereas the ordinary half-coke from mineral coal develops only small quantities of gas under the same conditions.

The working of the tar extracting apparatus may be carried through continuously without forming considerable quantities of decomposition gases in the gases free of oxygen which are used for the separation of the 100 tar.

One example of carrying the method into effect is as follows:

Gases free of oxygen, consisting of generator gases or produced from other suitable substances, are carried through a well insulated shaft of about 3 metres in height by introducing said gases at the lower end of the shaft at an initial temperature of about 500° C. The quantity of the gases must be so calculated that to 1 kg. of mineral coal to be freed of tar, at least 5-6 cubic metres of the hot gas mixture are used. In that operation the coal is charged continuously in opposition to the gas current. The gases, laden with tar vapours, leave the upper end of the shaft at a temperature of about 100° C. and are then cooled in a suitable device and freed of tar and partially returned into the process whereby they are first used for cooling the flame-coke freed of tar and then mixed with the hot gases so that their

quantity and temperature are in accord with the aforesaid conditions.

The quantity of gas, as herein given in cubic meters and kilogrammes (5-6 m.<sup>3</sup> per one kg. of mineral coal) is equal to 80-96 cubic feet per pound of coal.

Having now particularly described and ascertained the nature of my said invention and in what manner the same is to be performed, I do declare that what I claim is:

A method for the production of coke and tar from coal, which consists in subjecting mineral coal in the form of a continuously downwardly travelling column in counter-current to the action of gases free from oxygen at a rate of at least 80-96 cubic feet of gas per pound of mineral coal and at a temperature of the gas of about 500° C.

In testimony whereof I hereunto affix my signature.

FRITZ SEIDENSCHNUR.